

1

2,749,260

## FABRICATION OF RHENIUM

Chester T. Sims, Worthington, Ohio, assignor, by mesne assignments, to The Battelle Development Corporation, Columbus, Ohio, a corporation of Delaware

No Drawing. Application April 28, 1954,  
Serial No. 426,291

10 Claims. (Cl. 148—11.5)

This invention relates to a method of fabricating rhenium metal. More particularly, it relates to a process for producing rhenium metal sheet or wire by a combination of cold-working and annealing steps.

Rhenium metal is characterized by the fact that it is difficult to work and fabricate. It is exceedingly hot short, apparently because of low-melting rhenium heptoxide present at the grain boundaries. Since this oxide melts at 297° C., all attempts to hot work rhenium have failed. Furthermore, past efforts to alternately cold work and anneal rhenium have failed because the metal cracks up early in the cold-working process. Consequently, all previous attempts to provide a method for reducing rhenium ingots or bars to sheet or wire form have not been successful and the metal has generally been considered to be incapable of being fabricated on a practical basis.

It is, therefore, an object of this invention to provide a method for fabricating rhenium metal.

It is another object of this invention to provide a practical method or process for preparing rhenium metal sheet or wire.

Other objects and advantages of the present invention will be apparent in view of the following detailed description thereof.

In general, this invention comprises a method of fabricating rhenium metal comprising the steps of subjecting the rhenium metal to a number of mild cold-working operations with intermediate annealing steps, then subjecting the metal to more severe cold-working operations with longer time intermediate annealings.

It has now been found that rhenium metal bars and ingots can be reduced to sheet or wire form by a series of cold-working operations with frequent intermediate annealing treatments. For purposes of illustration, this process will hereinafter be described in terms of specific procedures. However, it will be apparent that the invention is not limited to such specific procedures, but is to be interpreted more broadly in accordance with the general description above.

Rhenium bars having a square or rectangular cross section may be prepared by pressing, presintering and sintering rhenium metal powder in accordance with well-known powder metallurgy techniques. It has been found to be desirable and preferable to first work such bars into a generally octagonal cross-section form, if a final round form, such as rod or wire, is desired. This is readily accomplished by first performing a hand-forging or hammering operation along the edges of the bar to flatten the corners of the original bar. An annealing treatment at a temperature in the range of from 1600–1800° C. for a period of from 20 to 40 minutes should follow this hand-forging operation. Both steps should be repeated once or twice to effect a total reduction of about 12% on the transverse diagonal of the bar. A cold-rolling

2

operation to smooth the original faces of the bar should follow. This will produce a negligible reduction in thickness or area. Further cold rolling along the edges of the bar to octagonize the bar is next recommended. Two or three such operations, with intermediate annealing treatments at 1600–1800° C. for 20 to 40 minutes, should provide a completely octagonized bar and effect an additional 5–8% reduction in length of the diagonal per cycle. From this point on, reductions of 10–20% in cross-sectional area per cold-working operation are preferable, although reductions of a number of cold-swaging steps, each producing 10–20% area reduction and with intermediate annealing treatments at 1600–1800° C. for 50–130 minutes may be used. The surface hardness values should be reduced to less than 300 Vickers hardness number by each annealing step. If wire is to be made from the rhenium bar, cold-drawing operations after a few swaging operations to reduce the area by 10–20% and with intermediate anneals for 50–130 minutes at 1600–1800° C. are permissible.

If it is desired to produce rhenium sheet rather than rod or wire, the octagonization step, as described above, is not necessary. Instead, a hand-forging or hammering operation is performed along the edges and sides of the bar to be cold rolled to sheet. An annealing treatment at a temperature in the range of from 1600–1800° C. for a period of from 20–40 minutes should follow the hand-forging operation. Cold rolling is then performed so as to reduce the thickness of the bar by about 2% per pass, each pass being followed by an annealing treatment at a temperature in the range of from 1600–1800° C. for a period of from 20–40 minutes. These rolling and annealing operations are repeated about five times, so as to obtain a total reduction of the bar of about 10% in thickness. Next, heavier cold-rolling passes are employed to reduce the bar to the desired sheet thickness. These passes are carried out in such a way as to reduce the bar by about 10% per pass, each pass being followed by an annealing treatment of from 110–250 minutes at a temperature of from 1600–1800° C. The surface-hardness values should be reduced to less than 350 Vickers hardness number by the annealing.

In general, it is possible to provide rhenium metal rods, wires, sheets, or other forms by a process comprising light cold-working operations followed by annealing, followed, in turn, by more severe cold-working operations such as cold rolling, cold swaging, cold wire-drawing, cold forging, cold rod-rolling, cold Turk's Head rolling, etc., or any combination of such cold-working processes.

As an example of the operation of the present method, the following data showing the dimensions prior to and following each cold-working and annealing step for the preparation of round rhenium rod are submitted. These data are exemplary only, and not restrictive or definitive of the scope of the process.

*Example*

60 A rhenium bar, 0.204-inch on a side, having 0.288-inch diagonals, was hand hammered to produce 0.270-inch diagonals (6% reduction in diagonal length), then annealed for 30 minutes at 1700° C., hand hammered to 0.261-inch diagonals (3% reduction), and annealed again 65 for 30 minutes at 1700° C. This edge-forging operation changed the side dimensions of the bar to 0.205 inch and 0.207 inch, respectively.

The bar was next cold rolled (roll setting 0.195 inch one pass on each side, producing side dimensions of 0.204 and 0.205 (1% reduction in bar width), respectively.

The forged edges of the bar were then cold rolled to

octagonize the rhenium metal bar. The tabulation below indicates the progress of this operation:

| Roll Setting (inch) | Octagonal Thickness (inch) | Vickers Hardness | Annealing Time (Minutes) | Temperature (° C.) | Remarks      |
|---------------------|----------------------------|------------------|--------------------------|--------------------|--------------|
| 0.220               | 0.260-0.265                | 450              | ---                      | ---                | As received. |
|                     | 0.242-0.248                | 279              | 45                       | 1,700              | Reduced 7%.  |
| 0.215               | 0.220-0.224                | 322              | 120                      | 1,700              | Reduced 5%.  |
| 0.200               | 0.216-0.222                | ---              | ---                      | ---                | Reduced 6%.  |

The sides of the original square were then cold rolled (roll setting, 0.195 inch) to produce a thickness of 0.209 inch, and effect the smoothing of all eight sides.

At this point, the alternate cold-swaging and annealing steps were employed. The cold-swaging steps were calculated to effect a 20% reduction in cross-sectional area per pass. The alternate swaging and annealing steps were continued until the bar had been reduced to an 0.062-inch diameter wire. The following tabulation shows the step-by-step progress of this process:

| Dia Size (inch) | Diameter (inch) | Vickers Hardness | Annealing      |                    |
|-----------------|-----------------|------------------|----------------|--------------------|
|                 |                 |                  | Time (Minutes) | Temperature (° C.) |
| 0.210-0.220     | 0.227           | 227              | 120            | 1,700              |
| 0.208           | 0.219           | 519              | 120            | 1,700              |
| 0.171           | 0.183           | 526              | 120            | 1,700              |
| 0.153           | 0.166           | 618              | 120            | 1,700              |
| 0.136           | 0.147           | 300              | 120            | 1,700              |
| 0.121           | 0.133           | 280              | 120            | 1,700              |
| 0.108           | 0.120           | 642              | 120            | 1,700              |
| 0.096           | 0.109           | 292              | 60             | 1,700              |
| 0.086           | 0.096           | 642              | 60             | 1,700              |
| 0.076           | 0.086           | 294              | 60             | 1,700              |
| 0.068           | 0.078           | 681              | 60             | 1,700              |
| 0.060           | 0.075           | 281              | 60             | 1,700              |
| 0.057           | 0.067           | 314              | 60             | 1,700              |
| 0.057           | 0.067           | 279              | 120            | 1,700              |
| 0.057           | 0.066           | 287              | 120            | 1,700              |
| 0.057           | 0.065           | 279              | 60             | 1,700              |
| 0.057           | 0.063           | 280              | 60             | 1,700              |
| 0.057           | 0.062           | 279              | 60             | 1,700              |

<sup>1</sup> Bar cut into halves.

As has been mentioned previously, rhenium work hardens exceedingly rapidly. In fact, rhenium work hardens to a greater extent than any other metal whose properties are generally known. For this reason, rhenium metal has always developed cracks early in cold-working procedures. Now, however, a method of fabricating rhenium metal has been provided by this invention. The method requires that the initial cold-working operations be such as to produce only a mild effect on the metal. In this way, it is believed that the surface grain structure is refined with a consequent increase in strength and without subjecting the underlying metal to great stress. In this manner, a crack-resistant outer skin of refined metal is established so that the tendency of rhenium to edge-crack is overcome. Thus, after a number of cycles of mild cold working and intermediate annealing treatment, the metal is subjected to more severe cold-working operations with longer time intermediate annealings so that the metal is reduced to the desired final fabricated form.

The example above and the preceding descriptive matter show that rhenium metal can be worked and fabricated without destruction of the piece being fabricated, provided the working operations are cold-working operations and are carried out to effect only mild dimensional changes initially. In addition, frequent intermediate annealing treatments are required. By such methods, rhenium metal has been fabricated to form sheets, rods, and wire. So far as is now known, this is the first method to provide a successful way of fabricating rhenium metal.

A new and useful method of preparing fabricated rhenium metal having been hereinbefore generally and specifically described, it will be apparent that various modifications in the exact procedure may be effected without departing from the scope of the invention as set forth in the following claims.

What is claimed is:

1. A method of fabricating rhenium metal comprising the steps of subjecting the rhenium to a series of cold-work reductions mild enough to effect refinement of only the surface grain structure and thereby provide a crack-resistant outer skin of refined metal, annealing the metal following each such cold-work reduction, and then subjecting the metal to more severe cold-work reductions with intermediate anneals until the desired fabrication is achieved.

2. The method of claim 1 wherein said severe cold-work reductions operate to effect reductions of the order of 5-20% per operation.

3. The method of claim 1 wherein annealing treatments intermediate the severe cold-work reductions are carried out at a temperature in the range of from 1600°-1800° C.

4. The method of claim 1 wherein the severe cold-work reductions effect reductions of the order of 5-20% per operation and wherein the annealing treatments intermediate said severe reductions are carried out at a temperature in the range of from 1600°-1800° C.

5. A method of fabricating rhenium metal comprising the steps of subjecting the metal to a series of mild cold-working operations such as to effect a refinement of only the surface grain structure and thereby provide a crack-resistant outer skin, annealing the metal following each such cold-work reduction, then subjecting the metal to a series of severe cold-working operations with intermediate annealing treatments sufficient to reduce the surface hardness of the metal below 350 Vickers hardness number.

6. A method of fabricating rhenium metal comprising the steps of subjecting the metal to a series of mild cold-working operations such as to effect a refinement of only the surface grain structure and thereby provide a crack-resistant outer skin, annealing the metal following each such cold-working operation, then subjecting the metal to a second series of cold-working operations wherein reductions of 5-20% are effected, said cold-working operations being performed alternately with annealing treatments sufficient to reduce the surface hardness of the metal below 350 Vickers hardness number.

7. The method of claim 6 wherein the annealing treatments are performed at a temperature in the range of 1600°-1800° C. for a period of time sufficient to produce a surface hardness less than 350 Vickers hardness number.

8. The method of claim 6 wherein the annealing treatments are performed at a temperature in the range of 1600°-1800° C. for a period of from at least 20-40 minutes.

9. The method of claim 6 wherein said second series of cold-working operations effects reductions of 5-20% in the cross-sectional area of the metal.

10. A method of fabricating rhenium metal comprising the steps of subjecting the rhenium to a series of cold-work reductions mild enough to effect a refinement of only the surface grain structure and thereby provide a

5

crack-resistant outer skin, annealing the metal at a temperature of 1600°-1800° F. for 20 to 40 minutes following each such cold-work reduction, subjecting the metal to severe cold-work reductions of the order of 5-20% per operation, and intermediate these severe cold-work operations annealing the metal at a temperature of 1600°-1800° F. for a period sufficient to reduce the surface

6

hardness of the metal below 350 Vickers hardness number, and continuing alternate cold-work reduction and annealing until the desired dimensions are obtained.

5 References Cited in the file of this patent  
"Materials and Methods," March 1954, pages 88-91.